

C. J. REED.

PROCESS OF RECOVERING METALS.

APPLICATION FILED AUG. 25, 1915.

1,200,025.

Patented Oct. 3, 1916.

Fig. 1.



Fig. 2.



Fig. 3.



Inventor:

Charles J. Reed,  
Bynes Townsend & Buckminster,  
Attn: M. S.

# UNITED STATES PATENT OFFICE.

CHARLES J. REED, OF GLENSIDE, PENNSYLVANIA.

## PROCESS OF RECOVERING METALS.

1,200,025.

Specification of Letters Patent.

Patented Oct. 3, 1916.

Application filed August 25, 1915. Serial No. 47,313.

*To all whom it may concern:*

Be it known that I, CHARLES J. REED, a citizen of the United States, residing at Glenside, in the county of Montgomery and State of Pennsylvania, have invented 5 certain new and useful Improvements in Processes of Recovering Metals, of which the following is a specification.

My invention relates to the recovery of 10 metals from ores and other materials by electrochemical operations on aqueous solutions containing the metals.

In United States Letters Patent No. 699,414 and No. 699,415, patented May 6, 15 1902, I have described a method and apparatus for manufacturing caustic alkali through the electrolytic reduction and deposition of an alkali metal in a cathode of mercury and the subsequent electrolytic 20 dissolving of the alkali metal as an anode in a separate receptacle to an alkali hydroxid, the concentration of which tends to continuously increase. In the process herein described, which is not applicable 25 to alkali metals nor to any metal which cannot be electrolytically deposited in the metallic state from an aqueous solution without simultaneously amalgamating or alloying with mercury, I reduce in a first operation the recoverable metal from an aqueous 30 solution to the metallic state as an amalgam, or alloy in a cathode of metallic mercury, and by a subsequent operation in a separate receptacle I dissolve the recovered metal 35 from the amalgam as an anode into another solution and simultaneously deposit the recovered metal in a free and purified condition on a cathode of the same metal or a cathode of some other suitable conductor 40 with which it does not form an alloy or amalgam, while compensating for the metal dissolved by local or chemical action in the manner described below. This separate operation requires the transfer of the amalgam 45 first formed to a separate solution and practically to a separate receptacle. This transfer of the amalgam to the separate receptacle in a continuous and practical manner can be accomplished without at the same 50 time transferring the electric current by means of the apparatus described by me in United States Letters Patent No. 699,415, above referred to. In this separate receptacle, into which the amalgam has been 55 transferred, and in which it acts as an anode, I provide a suitable solution of the

same recoverable metal, into which the metal continuously dissolves from the amalgam now acting as anode and from which the metal is continuously deposited in the 60 metallic state free from mercury and other impurities on a cathode of the same metal or on a cathode of any suitable conductor with which it does not alloy. In this second electrolyte there is no continuous increase or concentration of the recoverable metal, because it is being deposited at the cathode at substantially the same rate as that at which it is dissolving at the anode. These operations enable me completely to 70 remove a highly electropositive metal, like zinc, iron, cobalt, nickel and others, from an acid solution, leaving the acid pure, and at the same time separating the metal in the pure metallic state. This process I find 75 is adapted to the recovery of any metal which is electropositive to mercury and dissolves electrolytically from an amalgam without dissolving the mercury, and is at the same time sufficiently electronegative in 80 character to be deposited in the free metallic state from a neutral or nearly neutral aqueous solution on a conductor with which it does not alloy or amalgamate. The principal metals to which I refer and which stand in this relation to the other metals, are zinc, iron, nickel, cobalt, cadmium, lead, 85 copper and some others. The process is particularly advantageous in its application to zinc, iron, nickel and cobalt, because these 90 metals are not so easily recovered by the methods heretofore in use.

My process may be carried out by the use of the apparatus described in U. S. Letters Patent No. 699,415, above referred to, or by 95 the apparatus hereinafter described.

For a full understanding of my invention, reference is made to the accompanying drawings, wherein—

Figure 1 is a central longitudinal section of an electrolytic apparatus for carrying the process into effect; Fig. 2 is a similar section of a supplemental amalgam-producing electrolytic cell; and Fig. 3 is a central longitudinal section of an apparatus for distilling the amalgam in a current of an inert gas.

Referring to Fig. 1, 1 represents a receptacle of non-conductive material, subdivided by a non-conductive partition 2, terminating above the bottom but below the surface of the amalgam to leave an aperture 3. 4 rep-

resents the insoluble anode, which may be of carbon or lead, and 5 a cathode which is preferably of the metal which is to be deposited. 6 represents a deposit of pure 5 metal. 7 is the amalgam in process of constant formation, and 8 is the amalgam functioning as anode in relation to the cathode 5. 9 is an aqueous solution of the metal to be recovered, for example a chlorid or sulfate 10 solution; and 10 is an aqueous solution of the said metal, this latter solution remaining in substantially constant condition as regards composition, concentration, and condition of acidity or neutrality.

15 Most if not all of the metals above mentioned to which the process is applicable have the property of dissolving slowly from an amalgam by local or purely chemical action into the solution of the same metal in 20 contact with the amalgam. If this tendency were not counteracted, the final result would be that the metal deposited in the cathode 7 would not be sufficient to supply this local or chemical dissolving and also to transmit 25 the total current to the cathode 5. In a series arrangement of this kind, therefore, it is necessary to supply some additional amalgam from time to time: this may be produced in an independent depositing cell, 30 such as that shown in Fig. 2, in which additional amalgam is prepared by electrolyzing an aqueous solution 9', as the sulfate or chlorid of zinc, etc., between an insoluble anode 4', and a mercury cathode 7'. As additional amalgam is supplied or transferred 35 to the receptacle 1, without transferring the current, the excess of depleted mercury must also be removed from this receptacle 1 without transferring the current.

40 It is not necessary to use the same salt of the metal in both receptacles. For example, I may use zinc sulfate in one and zinc chlorid in the other.

My process is applicable to the recovery 45 of zinc from the ore as solution of sulfate or chlorid, and also for the recovery of iron, nickel or cobalt from their ores.

The amalgam or alloy of recoverable metal with mercury, formed as above described, 50 may also be separated into free metallic mercury and the free metal by passing hydrogen or other reducing or inert gas through the melted alloy at a temperature high enough to expel the mercury. The apparatus shown 55 in Fig. 3 may be used for this purpose. It comprises a crucible 11 in which the alloy or amalgam is melted, provided with a cover 12 tightly fitting and excluding the air, also with an outlet tube 13, for the escape of the

inert gas and vapor of the mercury, and 60 with an inlet tube 14 for the introduction of the gas below the surface of the melted metal or alloy. The crucible, charged with the alloy, is heated to a temperature at which the alloy melts, and the gas is then passed 65 through the apparatus and circulated by means of a blower 15 through a condenser 16, in which the mercury condenses. The temperature is gradually increased until practically all of the mercury is removed 70 and collected in the condenser. The mercury may be contaminated with some of the recovered metal, but that will not be detrimental to the cyclical working of the process, inasmuch as this mercury is used again 75 to produce an amalgam of the same metal.

While in one of the claims specific reference is made to the recovery of zinc, it is to be understood that other metals which are electropositive to mercury, are capable 80 of dissolving electrolytically from the amalgam without solution of the mercury and are capable of being electrodeposited from neutral or slightly acid solutions upon a cathode with which they do not alloy or amalgamate 85 during the electrodeposition, the principal examples of such other metals being iron, nickel and cobalt, are to be regarded as equivalents of zinc for the purposes of this invention.

I claim:

1. The process of recovering metals which are electropositive to mercury from an aqueous solution, which consists in electrodepositing the metals in a cathode of mercury, dissolving said metal from the resulting amalgam and simultaneously depositing it upon a cathode with which it does not alloy or amalgamate, and compensating the solution of metal by local action from the 95 amalgam anode by supplying thereto the requisite additional quantities of amalgam.

2. The process of recovering zinc from its aqueous solutions, which consists in electrodepositing the metal in a cathode of mercury, dissolving the zinc from the resulting amalgam and simultaneously depositing it on a cathode with which it does not alloy or amalgamate, and compensating the solution of metal by local action from the amalgam anode by supplying thereto the requisite additional quantities of amalgam.

In testimony whereof I affix my signature in presence of two witnesses.

CHARLES J. REED.

Witnesses:

D. M. SWEENEY,  
P. J. SWEENEY.